

## UNITED STATES PATENT OFFICE

2,233,265

## MAGNESIUM BASE ALLOY

John C. McDonald, Midland, Mich., assignor to  
The Dow Chemical Company, Midland, Mich.,  
a corporation of Michigan

No Drawing. Application December 26, 1939,  
Serial No. 311,002

3 Claims. (Cl. 75—168)

The invention relates to magnesium base alloys and more particularly concerns an alloy of this nature having a high degree of formability associated with other desirable physical properties, such as good tensile and yield strengths.

Magnesium alloys are being widely used in various structural and mechanical arts where a light-weight metal is highly desirable, such as for use in making castings, forgings, and the like. However, the use of these alloys in the rolled form to make sheet metal articles requiring forming operations, such as bending, drawing, and the like, has not progressed as rapidly due to the fact that in general alloys having good formability, permitting relatively sharp bends to be made without the article developing external cracks, usually have inferior strength characteristics.

It is, accordingly, the principal object of the invention to provide a magnesium base alloy which can be made into rolled sheet or the like, possessing sufficient ductility or formability to be sharply bent, drawn, or otherwise shaped while having good tensile and yield strengths.

Other objects and advantages will be apparent as the description of the invention proceeds.

My invention resides in the discovery that a magnesium base alloy composed of from 0.3 to 10 per cent of silver, 1 to 15 per cent cadmium, 0.3 to 10 per cent aluminum, and from 0.01 to 1 per cent of calcium, the balance being substantially all magnesium, is endowed with the aforementioned properties. While the properties of good formability or ductility associated with high tensile and yield strengths are manifest over the entire range of composition indicated, I have found that in general the preferred combination of properties, such as the most desirable ductility for forming operations, coupled with exceptionally high tensile strength and yield strength, is obtained when the alloy contains from 0.5 to 5 per cent of silver, from 4 to 8 per cent of cadmium, 0.1 to 0.3 per cent of calcium, and from 1 to 5 per cent aluminum.

The specific proportion of each alloying metal and the total amount of the added alloying metals to be employed in the new alloy depends upon the use for which the alloy is intended. In general, it is preferable that the alloys contain more than about 75 per cent of magnesium and less than 25 per cent of the added metals. For example, in alloys where exceptionally good ductility or formability associated with high yield and tensile strengths is of principal im-

portance, the total added metals should not materially exceed 10 per cent; while in those instances where exceptionally high yield and tensile strengths are desirable, the total added metals may amount to as much as 15 per cent.

The following table lists some of the properties of rolled sheet metal made from my new quinary alloy and compares these properties with those of rolled sheet made from related quaternary alloys. A comparison of the properties illustrates the improvement of the strength characteristics of the new alloy over that of the closely related alloys. In the table the per cent elongation is to be regarded as a measure of the ductility or formability of the specimen.

Table

| Nominal composition in percent (remainder=magnesium) |     |     |     | Annealed                       |                                  |                                |
|------------------------------------------------------|-----|-----|-----|--------------------------------|----------------------------------|--------------------------------|
| Ag                                                   | Al  | Cd  | Ca  | Yield strength in lbs./sq. in. | Tensile strength in lbs./sq. in. | Percent elongation in 2 inches |
| —                                                    | 0.8 | 5.1 | 0.3 | 21,000                         | 34,000                           | 17                             |
| 1.0                                                  | 1.0 | —   | 0.3 | 18,000                         | 34,000                           | 14                             |
| 1.0                                                  | 0.9 | 4.7 | 0.3 | 22,000                         | 36,000                           | 18                             |
| 0.7                                                  | 5.2 | —   | 0.3 | 21,000                         | 38,000                           | 11                             |
| 0.9                                                  | 5.3 | 5.0 | 0.3 | 21,000                         | 39,000                           | 15                             |
| —                                                    | 0.8 | 9.3 | 0.3 | 18,000                         | 34,000                           | 13                             |
| 1.0                                                  | 1.0 | —   | 0.3 | 18,000                         | 34,000                           | 14                             |
| 1.0                                                  | 0.8 | 9.7 | 0.3 | 17,000                         | 34,000                           | 18                             |
| —                                                    | 6.0 | 8.6 | 0.3 | 23,000                         | 40,000                           | 10                             |
| 0.7                                                  | 5.2 | —   | 0.3 | 21,000                         | 38,000                           | 11                             |
| 1.0                                                  | 6.2 | 9.0 | 0.3 | 28,000                         | 43,000                           | 14                             |

The properties listed in the above table under the section headed by the term "annealed" were obtained by first rolling the alloys at a temperature between about 600° to 700° F. and thereafter annealing them at various temperatures in the temperature range from 400° to 800° F. The properties selected for the table were those of the annealed specimens which exhibited the maximum elongation.

By comparison of the properties listed in the above table, it will be observed that the combined properties of my new polynary alloy are superior to those of the quaternary alloys having similar percentages of alloying ingredients. For example, it will be noted that the composition containing lower percentages of alloying ingredients have improved elongation coupled with superior yield and tensile properties in the annealed state; while those having higher percentages of alloying ingredients show superior strength characteristics as well as good elongation or formability. Similarly, improvements will be noted through-

out the range of alloying ingredients indicated.

While the new alloy is most useful in the wrought form, such as sheets, due to its formability characteristics, it may also be suitably used in making castings, forgings, extruded forms, and the like. It is further pointed out that my new alloy is amenable to solution and precipitation heat treatments, which, accordingly, modify its properties.

- 10 The new alloy may be compounded in any of the ways known in the art, such as by adding the ingredients to molten magnesium under suitable flux. The flux should be substantially free from magnesium chloride, if the calcium content is 15 to be above 0.3 per cent. In those instances where the alloy is to be compounded containing less than 0.3 per cent of calcium, magnesium chloride may be present in the flux without exerting undue deleterious effects, but in this case 20 it is usually preferable to add the calcium last

without too much stirring or agitation in order that the loss of calcium in the flux will be substantially prevented.

I claim:

1. A magnesium base alloy containing from 0.3 to 10 per cent of silver, 1 to 15 per cent of cadmium, 0.3 to 10 per cent of aluminum, and from 0.01 to 1 per cent of calcium, the balance being magnesium.
2. A magnesium base alloy containing from 0.3 to 10 per cent of silver, 1 to 10 per cent of cadmium, 0.3 to 10 per cent of aluminum, and from 0.01 to 1 per cent of calcium, the balance being magnesium.
3. A magnesium base alloy containing from 1 to 5 per cent of silver, from 4 to 8 per cent of cadmium, from 1 to 5 per cent of aluminum, and from 0.1 to 0.3 per cent of calcium, the balance being magnesium.

JOHN C. McDONALD.